

# United States Patent

[11] 3,622,339

[72] Inventors Fumihiko Nishio;  
Nobuo Yamamoto; Jun Hayashi, all of  
Minami-Ashigara Machi, Ashigara-  
Kamigun Kanagawa, Japan

[21] Appl. No. 743,007

[22] Filed July 8, 1968

[45] Patented Nov. 23, 1971

[73] Assignee Fuji Shashin Film Kabushiki Kaisha

[32] Priority July 7, 1967

[33] Japan

[31] 42/43765

[54] **POLYMERIC ANTIFOGGANT CONTAINING AT LEAST FOUR TRIAZINE RINGS**  
8 Claims, No Drawings

[52] U.S. Cl. 96/109,  
96/114

[51] Int. Cl. G03c 1/34,  
G03c 1/72

[50] Field of Search 96/109

[56] References Cited  
UNITED STATES PATENTS  
2,945,762 7/1962 Carroll et al. 96/109

## FOREIGN PATENTS

1,150,279 6/1963 Germany ..... 96/109

Primary Examiner—Norman G. Torchin

Assistant Examiner—Richard E. Fichter

Attorney—Sughrue, Rothwell, Mion, Zinn & Macpeak

**ABSTRACT:** A photographic silver halide light-sensitive element illustrating a marked reduction in fog which has a layer which contains a compound having a repeating unit represented by the following formula:



The specific moieties symbolically represented in the above formula are defined in the specification. The active antifogant illustrated above may be incorporated into a silver halide emulsion layer, a protective layer and in intermediate layer or the like.

**POLYMERIC ANTIFOGGANT CONTAINING AT LEAST  
FOUR TRIAZINE RINGS**

**BACKGROUND OF THE INVENTION**

**1. Field of the Invention**

The present invention relates to an improved photographic silver halide light-sensitive element containing an antifoggant.

**2. Description of the Prior Art**

By incorporating in a photographic silver halide emulsion a natural active gelatin, a compound having labile sulfur, a noble metal salt, a heavy metal salt, reducing agents such as an amine, a hydrazine, or a polyalkylene oxide derivative, or combinations thereof, the sensitivity of the silver halide emulsion can be increased. However, fog tends to increase with the addition of such compounds. This tendency is increased as the period of time for storing photographic light-sensitive elements becomes longer, or the temperature and humidity during storage are increased.

In order to prevent the formation of fog, it is necessary to use an antifoggant. Aging tests have usually been conducted to test the preservability of photographic light-sensitive elements under high temperature and high humidity. It is desirable that photographic light-sensitive elements be as stable as possible under high temperature and high humidity conditions, as these are frequently encountered in the tropics.

**SUMMARY OF THE INVENTION**

It has been found that a photographic light-sensitive element in which the formation of fog may effectively be prevented without a reduction in sensitivity may be obtained by the incorporation in a silver halide layer, a protective layer and an intermediate layer or the like, of a compound which contains a repeating unit represented by the following formula:



wherein R<sub>1</sub> represents a member selected from the group consisting of —OR,



where R and R' each represent a member selected from the group consisting of (i) a hydrogen atom; (ii) an alkyl group having from one to 12 carbon atoms, a hydroxyalkyl group, a sulfoalkyl group, a salt thereof, a carboxyalkyl group, a salt thereof, and an aralkyl group, each of said groups having from one to four carbon atoms in the main straight carbon chain thereof; (iii) an unsubstituted aryl group having from six to 12 carbon atoms, an aryl group having from six to 12 carbon atoms substituted by a member selected from the group consisting of a sulfo group, a salt thereof, a sulfoxyl group, a salt thereof, a hydroxyl group, an alkyl group having from one to four carbon atoms, an alkoxy group having from one to four carbon atoms, and a halogen atom; an unsubstituted cycloalkyl group, and a cycloalkyl group substituted by a member selected from the group consisting of a sulfo group, a salt thereof, a sulfoxyl group, a salt thereof, a hydroxyl group, an alkyl group having from one to four carbon atoms, an alkoxy group having from one to four carbon atoms, and a halogen atom; and (iv) a heterocyclic group; A represents a member selected from the group consisting of a polymethylene group having from four to five carbon atoms, and a polymethylene group having a heteroatomic group and forming a five to six membered ring together with a nitrogen atom; R<sub>2</sub>, R<sub>3</sub>, R<sub>4</sub>, and R<sub>5</sub> each represent a member selected from the group consisting of a hydrogen atom, an alkyl group having from one to four carbon atoms and a hydroxyalkyl

group; Y<sub>1</sub>, Y<sub>2</sub>, Y<sub>3</sub>, and Y<sub>4</sub> each represent a member selected from the group consisting of a polymethylene group having from two to 12 carbon atoms, a polymethylene group having from two to 12 carbon atoms substituted by a member

5 selected from the group consisting of an alkyl group having from one to four carbon atoms and a hydroxyalkyl group having from one to four carbon atoms, an arylene group having six to 12 carbon atoms, an arylene group having from six to 12 carbon atoms substituted by a member selected from the group consisting of a sulfo group, a salt thereof, a carboxyl

10 group, a salt thereof, an alkyl group having from one to four carbon atoms, an alkoxy group having from one to four carbon atoms and a halogen atom, a cycloalkylene group having from six to 12 carbon atoms, and a cycloalkylene group having

15 from six to 12 carbon atoms substituted by a member selected from the group consisting of a sulfo group, a salt thereof, a carboxyl group, a salt thereof, an alkyl group having from one to four carbon atoms, an alkoxy group having one to four carbon atoms and a halogen atom; Z represents a member

20 selected from the group consisting of a divalent heteroatom, a divalent heteroatomic group, and a hydrocarbon residual group having from one to two carbon atoms; and k and m each represents 0 or 1.

25 When the compound shown above is present in the silver halide emulsion layer, it is preferred that it be present in amounts from about 0.01 g. to about 50 g./1 mole of silver halide in the emulsion. When the compound shown above is added to a protective layer, it is preferred that the compound

30 be present in amounts from about 0.05 g. to about 250/1 kg. of gelatin in the layer. When the compound shown above is added to an intermediate layer, it is preferred that the compound be present in amounts from about 0.05 g. to about 250 g./1 kg. of gelatin in the layer.

35 A number of specific examples of the compound utilized in the present invention are set out in the specification, and various acceptable methods of forming the compound of the present invention are also illustrated therein.

An object of this invention is to provide a photographic 40 light-sensitive element in which the formation of fog is effectively prevented without a reduction in sensitivity.

Another object of this invention is to provide a photographic light-sensitive element which can be stored for a long period of time without the formation of fog and which will remain stable during storage.

Still another object of this invention is to provide a photographic emulsion having a good preservability, that is, one which will illustrate less degradation in sensitivity and contrast when preserved for a long period of time.

55 A still further object of this invention is to provide a photographic light-sensitive element in which the formation of fog, caused when the photographic silver halide emulsion layer is processed in a formalin-containing bath before developing in order to preliminarily harden the gelatin film, is prevented without lowering the sensitivity of the light-sensitive photographic element.

To prevent the formation of fog in photographic light-sensitive elements it has been found that the objects of this invention can be attained by incorporating in a photographic layer of a photographic light-sensitive element, having a silver halide emulsion layer, an antifoggant having a repeating unit represented by the following general formula (I):



70 75 70 where R<sub>1</sub> represents a member selected from the group consisting of



where R and R' each represents a member selected from the group consisting of (i) a hydrogen atom; (ii) an alkyl group having one to 12 carbon atoms, a hydroxyalkyl group, a sulfoalkyl group, a salt thereof, a carboxyalkyl group, a salt thereof, and an aralkyl group, each of said groups having from one to four carbon atoms in the main straight carbon chain thereof; (iii) an unsubstituted aryl group having from six to 12 carbon atoms, an aryl group having from six to 12 carbon atoms substituted by a member selected from the group consisting of a sulfo group, a salt thereof, a sulfoxyl group, a salt thereof, a hydroxyl group, an alkyl group having from one to four carbon atoms, an alkoxy group having from one to four carbon atoms, and a halogen atom; an unsubstituted cycloalkyl group, and a cycloalkyl group substituted by a member selected from the group consisting of a sulfo group, a salt thereof, a sulfoxyl group, a salt thereof, a hydroxyl group, each of said cycloalkyl groups having from three to six carbon atoms, an alkyl group having from one to four carbon atoms, an alkoxy group having from one to four carbon atoms, and a halogen atom; and (iv) a heterocyclic group; A represents a member selected from the group consisting of a polymethylene group having from four to five carbon atoms, and a polymethylene group having a heteroatomic group and forming a five- to six-membered ring together with a nitrogen atom; R<sub>2</sub>, R<sub>3</sub>, R<sub>4</sub> and R<sub>5</sub> each represent a member selected from the group consisting of a hydrogen atom, an alkyl group having from one to four carbon atoms and a hydroxyalkyl group; Y<sub>1</sub>, Y<sub>2</sub>, Y<sub>3</sub> and Y<sub>4</sub> each represent a member selected from the group consisting of a polymethylene group having from two to 12 carbon atoms, a polymethylene group having from two to 12 carbon atoms substituted by a member selected from the group consisting of an alkyl group having from one to four carbon atoms and a hydroxyalkyl group having from one to four carbon atoms, an arylene group having from six to 12 carbon atoms, an arylene group having from six to 12 carbon atoms substituted by a member selected from the group consisting of a sulfo group, a salt thereof, a carboxyl group, a salt thereof, an alkyl group having from one to four carbon atoms, an alkoxy group having from one to four carbon atoms and a halogen atom, a cycloalkylene group having from six to 12 carbon atoms, and a cycloalkylene group having from six to 12 carbon atoms substituted by a member selected from the group consisting of a sulfo group, a salt thereof, a carboxyl group, a salt thereof, an alkyl group having from one to four carbon atoms, an alkoxy group having from one to four carbon atoms and a halogen atom; Z represents a member selected from the group consisting of a divalent heteroatom, a divalent heteroatomic group and a hydrocarbon residual group having from one to two carbon atoms; k and m each may represent 0 or 1; R<sub>2</sub> may be same as R<sub>4</sub>; R<sub>3</sub> may be same as R<sub>5</sub>; Y<sub>1</sub> may be same as Y<sub>3</sub>; and Y<sub>2</sub> may be same as Y<sub>4</sub>.

The antifoggant used in the present invention is a high molecular compound having s-triazine rings prepared by the method described below.

Although there is no particular restriction about the distribution of polymerization degree, based on the viscosity of a solution of the antifoggant or the number of the terminal groups of said compound, the main component of the antifoggant is considered to be composed of a polymer having more than four s-triazine rings in the main chain.

The aforesaid antifoggant having a repeating unit represented by general formula (I) described above may be prepared by the polycondensation reaction of a s-triazine 65 compound represented by general formula (II):



(II) 75

[wherein X represents a halogen atom such as a chlorine atom or a bromine atom, R<sub>1</sub> has the same meaning described in connection with general formula (I) and a diamino compound, represented by general formula (III) or (IV)]

5



10



[wherein R<sub>2</sub>, R<sub>3</sub>, R<sub>4</sub>, R<sub>5</sub>, Y<sub>1</sub>, Y<sub>2</sub>, Y<sub>3</sub>, Y<sub>4</sub>, Z, k, and m have the same meaning as described in connection with general formula (I) or by the polycondensation reaction of a bis-(halogeno-s-triazine) compound represented by general formula (V) or (VI)]

20



25



[wherein X has the same meaning described in connection with general formula (II) and R<sub>1</sub>, R<sub>2</sub>, R<sub>3</sub>, R<sub>4</sub>, R<sub>5</sub>, Y<sub>1</sub>, Y<sub>2</sub>, Y<sub>3</sub>, Y<sub>4</sub>, Z, k and m have the same meaning as described in connection with general formula (I)] and the aforesaid diamino compounds represented by general formula (III) or (IV).

The halogeno-s-triazine compounds represented by general formulas (II), (V) and (VI) described above may be prepared from cyanuric chloride by the method described in the "Journal of the American Chemical Society"; Vol. 73, 2981-2992 (1951).

The antifoggants used in this invention will now be explained in greater detail.

Examples of R<sub>1</sub> aforesaid general formula (I) and general formulas (II), (V) and (VI), illustrating the starting materials, may be as follows:

-OH, -OCH<sub>3</sub>, -OC<sub>2</sub>H<sub>5</sub>, -OC<sub>4</sub>H<sub>9</sub>



70





## As examples of the groups



which occur in the compounds represented by general formulas (III), (IV), (V) and (VI), which are the starting materials for the antifogging agent represented by general formula (I), or the reagents in the polycondensation for preparing the antifogging agent of this invention, are illustrated as follows:



40 The preparation of the antifogging agent having a repeating unit represented by general formula (I) described above may be prepared by the following two illustrative general methods.

a. About 1 mole of the dihalogeno-s-triazine compound represented by general formula (II) is reacted with 1 mole of the diamino compound represented by general formula (III) or (IV) in a suitable solvent, preferably water, acetone, dioxane, dimethylformamide, or diethylformamide at a proper temperature, e.g., at about 10-150° C., with or without a suitable base preferably an alkali bicarbonate, an alkali carbonate, a caustic alkali, or an organic base, e.g., pyridine, 2,4,6-trimethylpyridine, and diamino-bicyclooctane; and

45 b. About 1 mole of the bis(halogeno-s-triazine) compound represented by general formula (V) or (VI) described above is reacted with one mole of the diamino compound represented by general formula (III) or (IV) at a suitable temperature (preferably 30-150° C.) in the solvent and, if desired, in the presence of a base as stated in method (a)

50 55 60 The antifogging agent of the present invention may, of course, be prepared by methods other than those described above.

Typical examples of a compound having a repeating unit represented by general formula (I) or (II) are illustrated below. The number of s-triazine rings







The above compounds may generally be prepared by method (a) or (b) described above by specific examples of methods of preparation of compound 1 and compound 2 will be described below.

Preparation of compound 1 (method a):

368 g. of cyanuric chloride dissolved in 1.1 liters of acetone was gradually added to 1.5 liters of water, cooled to a temperature lower than 10° C., with stirring. While further stirring the mixture at a temperature lower than 5° C., a solution consisting of 122 g. of ethanol amine, 212 g. of sodium bicarbonate and 800 ml. of water was added to the mixture over a 1.5 hour period. After additional stirring for 2 hours at the same temperature, the temperature of the mixture was gradually raised to about 15° C. The system was further stirred for an additional 1 hour at this temperature. Crystals precipitated, and were recovered by filtration and subsequently recrystallized from water containing a small amount of sodium bicarbonate to yield 253 g. of 2,4-dichloro-6-(2-hydroxyethylamino)-s-triazine. The product was a white crystal having a melting point of 117-119° C. (decomposed).

55 The 2,4-dichloro-6-(2-hydroxyethylamino)-s-triazine (209 g.) obtained was mixed with 2 liters of water and while stirring the mixture at a temperature of 20-25° C., a solution consisting of 70 g. of 1,3-diaminopropane and 300 ml. of water was added to the mixture over a one hour period. Thereafter, the temperature of the system was elevated to 30-35° C. and a solution consisting of 168 g. of sodium carbonate and 1 liter of water was added to the mixture over a 40-minute period. After the addition thereof, the temperature of the system was elevated gradually and stirred for 3 hours at 95-100° C. The reaction mixture was filtered after being allowed to cool, and the product thus recovered was washed with water, until the washings became neutral, and dried to provide 200 g. of the white powders of compound 1. The intrinsic viscosity of compound 1 measured in dimethylformamide at 35° C. was 0.104.

60 Preparation of Compound 2 (method b):

65 A mixture of 250 g. of 2,4-dichloro-6-(2-hydroxyethylamino)-s-triazine (prepared by the method described above,) 2 liters of acetone and 1 liter of water was stirred at 70 20° C. After adding a solution consisting of 40.7 g. of 1,3-

diaminopropane and 200 ml. of water to the mixture over a 30-minute period, a solution consisting of 101 g. of sodium carbonate and 1 liter of water was added thereto over a 30-minute period. After completing the addition, the temperature of the system was raised to 40-45° C., and the system was stirred for 1 hour. The reaction mixture was then ice-cooled and filtered to provide 232 g. of a white crystal. The product was recrystallized from a dioxane-water 1:1 mixed solution to provide 184 g. of the white crystal of 1,3-bis(2'-chloro-4'-hydroxyethylamino-s-triazine-6'-ylamino)-propane, having a melting point (decomposed) of 276°C.

A mixture of 42.5 g. of the 1,3-bis(2'-chloro-4'-hydroxyethylamino-s-triazine-6'-ylamino) propane thus obtained and 400 ml. of water was stirred at 30-35° C., and after adding a solution consisting of 7.4 g. of ethylenediamine monohydrate and 30 ml. of water to the mixture, the temperature of the resulting mixture was elevated to 40-45° C. Thereafter a solution consisting of 16.8 g. of sodium bicarbonate and 120 ml. of water was added to the mixture over a 30-minute period.

The temperature of the system was further elevated to 90-95° C., and heated and stirred for 3 hours. The reaction mixture was then cooled to room temperature, filtered, washed with water and dried to provide 40 g. of the white powders of compound 2. The intrinsic viscosity of the product in dimethylformamide, measured at 35°C., was 0.125.

Compounds 3-20, which are shown above as typical examples of the antifogants used in this invention, may be prepared by methods similar to those illustrated for preparing compound 1 and compound 2. To illustrate the excellent antifogging effect of the antifogant of this invention, the physical retardance of the antifogant of this invention compared with that of known antifogant is shown in the table below. In this table, the physical retardance value was observed by conventional physical retardance measuring methods for testing the chemical properties of photographic gelatin e.g., "Testing for Photographic Gelatin" (PAGI method); "Commission Testing Method for Photographic Gelatin (Japan)," 12-13 (1964). Specifically, the measurement was performed as in the PAGI method with the exception that each of the compounds was added to inert gelatin and employed as the sample. This measurement has been widely used, in view of the fact that the retardance in the 2nd ripening is proportional to the physical retardance of the silver halide particle growth. The numeral 10 in the table represents the maximum retardance, and the numeral 0 represents a sample having no inhibiting properties.

| Material*     | Physical Retardance | pH At Measurement |
|---------------|---------------------|-------------------|
| a Compound 1  | 9                   | 5.0               |
| b Compound 2  | 8                   | 5.0               |
| c Compound 3  | 6                   | 4.9               |
| d Compound 4  | 8                   | 4.9               |
| e Compound 9  | 7                   | 4.8               |
| f Compound 10 | 7                   | 4.9               |
| g Compound 11 | 8                   | 5.0               |
| h Compound 13 | 9                   | 4.8               |
| i Compound 14 | 9                   | 4.9               |
| j Compound 15 | 8                   | 4.8               |

|                                                                                            |   |     |
|--------------------------------------------------------------------------------------------|---|-----|
| k Compound 16                                                                              | 8 | 4.9 |
| l Compound 19                                                                              | 7 | 4.8 |
| m Compound 20                                                                              | 8 | 4.9 |
| n 5-Mercapto-1-phenyl-tetrazole                                                            | 9 | 5.0 |
| o 4-Hydroxy-6-methyl-1,3,3a,7-tetrazindene                                                 | 8 | 5.0 |
| p 2,4,6-Trihydroxy-s-triazine                                                              | 1 | 5.0 |
| q 2,4,6-Trihydroxyethyl-s-triazine                                                         | 0 | 5.0 |
| r 2,4-Dihydroxy-6-sulfoethylamino-s-triazine                                               | 0 | 5.0 |
| s 2-(3-Sulfoanilino)-6-hydroxy-4-(2-hydroxyethylamino-s-triazine)                          | 0 | 4.8 |
| t 1,4-Bis(4,6-di(2-hydroxyethylamino)s-triazine-2-ylamino)butane                           | 0 | 5.0 |
| u 4,4'-Bis[4-anilino-6-(2-hydroxyethylamino)s-triazine-2-amino]stilbene-2,2'-sulfonic acid | 0 | 5.0 |
| Control (no antifogging)                                                                   | 0 | 5.0 |

\* The concentration of the material used in the measurement was measured by adding 1.6 ml. of a 1 percent solution of each sample to 75 ml. of the test solution (corresponding to 0.34 g. of  $\text{AgNO}_3$ ).

As may be seen from the above table, compounds a-m of the present invention show physical retardance values in the range of compound n, 5-mercaptop-1-phenyltetrazole and compound o, 4-hydroxy-6-methyl-1,3,3a,7-tetrazindene, which are both known as excellent antifogants. The nonhigh molecular compounds (p-u shown above), which are similar to the antifogants of this invention in that they have one or two s-triazine rings, show a very weak physical retardance or lack of physical retardance.

The molecular size of the high molecular antifogant used in this invention, or, in other words, the number "n" of the s-triazine rings contained in compounds 1-20, will now be explained in greater detail. Although these high molecular antifogants may be prepared by the methods described above, reaction products prepared by the polycondensation reaction of a dihalogeno-s-triazine compound and a diamino compound are obtained as a mixture of polymers having different distributions of polymerization degree, depending upon reaction conditions, such as reaction time, reaction temperature, reaction solvent, the catalyst, if one is used, and the mole ratio of the dihalogeno-s-triazine compound to the diamino compound.

It has been found, however, that reaction products thus obtained show remarkable practical merit for use as antifogants, based on experimental results, only when the products consist mainly of compounds having more than four s-triazine rings as the repeating unit. To illustrate, each conventional control compound (compounds v-z) which have one or two s-triazine rings, and compound 1 ( $n=4$  or 11) of this invention, were added to a silver iodo-bromide high speed negative emulsion, which has been sulfur-sensitized and gold-sensitized. The antifogging effect and the physical inhibittance were then measured and the results are shown in the following table.

From the results of the above experiment, it was found that while the conventional compounds illustrated, at best, a very weak antifogging effect, compound 1, which is an example of the antifogant of the present invention, shows a very strong antifogging effect when the number of s-triazine rings was four, as well as when the s-triazine rings numbered 11.

| Compound | Concentration, g./Ag $\times 1$ mol | Relation sensitivity | Fog            | Physical inhibittance |
|----------|-------------------------------------|----------------------|----------------|-----------------------|
| v        | 2.0<br>4.0                          | 97<br>96             | 0.16<br>0.17 } | 0                     |
| w        | 2.0<br>4.0                          | 97<br>98             | 0.17<br>0.16 } | 0                     |



| x-----              |  |  | 2.0<br>4.0 | 97<br>96 | 0.18<br>0.17 } | 0 |
|---------------------|--|--|------------|----------|----------------|---|
| y-----              |  |  | 2.0<br>4.0 | 98<br>97 | 0.17 }         | 0 |
| z-----              |  |  | 2.0<br>4.0 | 96<br>95 | 0.16 }         | 1 |
| 1 (n=4)-----        |  |  | 2.0<br>4.0 | 99<br>98 | 0.12<br>0.08 } | 8 |
| 2 (n=11)-----       |  |  | 2.0<br>4.0 | 98<br>97 | 0.09<br>0.06 } | 9 |
| Control (none)----- |  |  |            | 100      | 0.17           |   |

The intrinsic viscosity  $[\eta]$  of compound 1 measured in DMF (n=4 or 11) at 35°C., and the values of elementary analysis thereof, were as follows:

|           | Chlorine |       | Nitrogen percent |       |            |
|-----------|----------|-------|------------------|-------|------------|
|           | $[\eta]$ | Found | Calculated       | Found | Calculated |
| n=4-----  | 0.058    | 8.72  | 8.46             | 36.77 | 36.65      |
| n=11----- | 0.120    | 2.98  | 3.08             | 38.52 | 38.80      |

The compound, having the repeating unit shown by general formula (I), used in this invention shows an excellent antifogging effect or stabilizing power for photographic silver halide light-sensitive elements, and does not harmfully influence any other useful photographic properties.

The compounds of the invention may be used alone (or as mixtures thereof) as antifogging agents or stabilizers. In addition, they may be used in combination with conventional antifog-

The antifogging agents of this invention may be added to the silver halide emulsion at stages before the emulsion is applied to a support, but is preferably added between after-ripening and coating. Further, it has been found that the antifogging agent of this invention can be very effectively incorporated in a photographic layer other than the silver halide emulsion layer, such as, a protective layer other than the silver halide emulsion layer, such as, a protective layer adjacent the silver halide emulsion layer or an intermediate layer between silver halide emulsion layers. In addition, since these compounds are dissolved in solvents such as water, dimethylformamide, dimethyl sulfoxide, water containing an acid (inorganic acids such as hydrochloric acid, sulfuric acid, nitric acid, etc. or organic acids such as acetic acid) or water containing an alkali (such as acid alkali carbonate, an alkali carbonate, or an alkali hydroxide), it is often desirable to add the antifogging agent in the form of a solution in the aforesaid solvents.

There is no particular limit to the concentration of the antifogging agent of this invention which may be used, but a suitable concentration is generally 0.01-50 g. per 1 mole of silver halide when incorporating it in a silver halide emulsion layer,

and 0.05-250 g. per 1 kg. of gelatin when adding it to a protective layer or to an intermediate layer.

The present invention is applicable to black and white negative emulsions, X-ray emulsions, the so-called coupler-in-emulsion-type color photographic silver halide emulsions, wherein a color coupler is incorporated in the emulsion, and the so-called coupler-in-developer-type color photographic silver halide emulsion, wherein a color coupler is incorporated in the developer. Improved results can be obtained when it is applied to a gelatino silver iodo-bromide emulsion. However, the invention is applicable to various other types of silver halide emulsions.

A silver halide emulsion containing the antifogging agent of this invention may be chemically sensitized by conventional methods, such as by the addition of a compound containing a labile sulfur, e.g., ammonium thiosulfate and allylthio urea (cf., if necessary, "The Theory of the Photographic Process", 3rd edition, 113-116 (1966); MacMillan Company, New York); a complex salt of monovalent gold and thiocyanic acid (ibid., page 116) reducing sensitizers, such as amines, hydrazines or a heavy metal salt such as stannous chloride (ibid.; pages 113-116); and polyalkylene oxide derivatives, or combinations thereof. The emulsion used in this invention may further contain an inorganic hardening agent (ibid., page 55); or an organic hardening agent (ibid., pages 55-60). Moreover, the silver halide emulsion in this invention may contain a wetting agent, for example, a nonionic surface active agent, such as polyoxyethylenenonylphenyl ether; an anion surface active agent such as sodium alkylbenzene sulfonate or sodium N-alkanoyl-N-alkyl taurate; an amphoteric surface active agent; or anionic surface active agent containing an ethylene oxide chain as described in Belgian Pat. No. 650,004.

The antifogging agent used in this invention having the repeating unit represented by general formula (I) has properties which differ from those of conventional antifogging agents in that the antifogging agent of this invention has a high molecular weight, and the antifogging agent of this invention shows excellent antifogging effects with respect to silver halide emulsions.

Various s-triazine-type antifogging agents (e.g., U.S. Pat. Nos. 75 2,476,536 and 2,948,612) have been known, but they were

low molecular compounds having one triazine ring, hence quite different from the high molecular weight antifoggants containing a plurality of s-triazine rings as in the present invention.

It is well known that it is difficult to prevent the formation of fog in a photographic silver halide emulsion, when the sensitivity of the emulsion has been increased by the combination of a sulfur sensitization, a gold sensitization and a reduction sensitization. The antifoggant of this invention can effectively prevent the formation of fog in a silver halide emulsion sensitized by the combination of the three sensitizing methods described, and this will be without substantially reducing the sensitivity of the silver halide emulsion.

The formation of fog in a photographic silver halide emulsion which has been subjected to a prehardening process by, e.g., formalin and the like, cannot be prevented. But, by using the antifoggant of this invention, such fog can be effectively prevented without harmful affects on photographic properties.

The invention will now be explained in greater detail by reference to the following examples.

#### EXAMPLE 1

Each of the antifoggants (1)-(5), (13), (16) and (17) was incorporated in a sulfur- and gold-sensitized, high-speed gelatin-silver iodobromide negative emulsion, respectively, and the resulting silver halide emulsions were applied to a film base and dried. The light-sensitive films thus prepared were exposed on an NSG II-type sensitometer (made by Tokyo Shibaura Electric Co.) and developed in a developer having the following composition for 8 minutes at 20° C:

|                                |          |
|--------------------------------|----------|
| N-methyl-p-aminophenol sulfate | 2 g.     |
| Sodium Sulfite (anhydrous)     | 100 g.   |
| Hydroquinone                   | 5 g.     |
| Borax                          | 2 g.     |
| Water to make                  | 1 liter. |

The photographic properties of the developed photographic films were examined and were compared with those of photographic films prepared and developed under same conditions except that the antifoggant of this invention was not included. The results of this experiment are shown in the following table.

|                   | Concentration<br>(g./Ag 1 mol) | Fresh          |                | After aging <sup>a</sup> |      |
|-------------------|--------------------------------|----------------|----------------|--------------------------|------|
|                   |                                | A <sup>1</sup> | B <sup>2</sup> | A                        | B    |
| None (control)    | 100                            | 0.14           |                | 75                       | 0.27 |
| Anti-foggant (1)  | 0.4                            | 100            | 0.11           | 95                       | 0.16 |
|                   | 0.8                            | 97             | 0.09           | 90                       | 0.11 |
| Anti-foggant (2)  | 0.4                            | 98             | 0.10           | 98                       | 0.14 |
|                   | 0.8                            | 95             | 0.07           | 92                       | 0.11 |
| Anti-foggant (3)  | 3.0                            | 102            | 0.12           | 94                       | 0.18 |
|                   | 6.0                            | 97             | 0.11           | 90                       | 0.15 |
| Anti-foggant (4)  | 0.8                            | 98             | 0.09           | 93                       | 0.13 |
|                   | 1.6                            | 94             | 0.07           | 88                       | 0.09 |
| Anti-foggant (5)  | 0.8                            | 98             | 0.12           | 96                       | 0.19 |
|                   | 1.6                            | 98             | 0.10           | 95                       | 0.14 |
| Anti-foggant (13) | 0.4                            | 96             | 0.10           | 90                       | 0.12 |
|                   | 0.8                            | 90             | 0.08           | 88                       | 0.09 |
| Anti-foggant (16) | 0.4                            | 96             | 0.11           | 96                       | 0.17 |
|                   | 0.8                            | 95             | 0.09           | 94                       | 0.13 |
| Anti-foggant (17) | 0.4                            | 101            | 0.13           | 90                       | 0.16 |
|                   | 0.8                            | 97             | 0.09           | 90                       | 0.11 |

<sup>1</sup> Relative sensitivity.

<sup>2</sup> Fog.

<sup>3</sup> After aging of 2 days at 50° C. at 80% relative humidity.

As shown by the above results, the initial formation of fog was prevented by the antifoggants of this invention, and when the photographic film was developed after being aged for 2 days at 50° C. and at a relative humidity of 80 percent, the formation of fog was also prevented, without a reduction in sensitivity.

#### EXAMPLE 2

Each of the antifoggants (6), (9), (10), (14) and (15) was incorporated in a sulfur-reduction-and gold-sensitized high-speed gelatin-silver iodobromide X-ray emulsion, respectively, and the resulting silver halide emulsion was applied to a film base. The light-sensitive films thus prepared were exposed on an NSG II-type sensitometer and developed for 6 minutes at 20° C. in a developer having the following composition:

|                                |          |
|--------------------------------|----------|
| N-methyl-p-aminophenol sulfate | 2 g.     |
| Sodium sulfite (anhydrous)     | 80 g.    |
| Hydroquinone                   | 8 g.     |
| Sodium carbonate (anhydrous)   | 40 g.    |
| Potassium bromide              | 2.       |
| Water to make                  | 1 liter. |

The properties of the developed film were compared with those of a photographic film treated under the same conditions with the exception that an antifoggant of this invention was not added. The results obtained are illustrated in the following table. From the results it is clear that the formation of fog was inhibited by the incorporation of the antifoggant of this invention when compared to the films wherein the antifoggant of this invention was not added.

| Concentration<br>(g./Ag 1 mol) | Relative<br>sensitivity | Fog  |
|--------------------------------|-------------------------|------|
| None (control)                 | 100                     | 0.23 |
| Antifoggant (6)                | 2.0                     | 0.20 |
| do                             | 4.0                     | 0.17 |
| Antifoggant (9)                | 0.8                     | 0.21 |
| do                             | 1.6                     | 0.18 |
| Antifoggant (10)               | 0.8                     | 0.19 |
| do                             | 1.6                     | 0.17 |
| Antifoggant (14)               | 0.8                     | 0.17 |
| do                             | 1.6                     | 0.13 |
| Antifoggant (15)               | 0.8                     | 0.20 |
| do                             | 1.6                     | 0.17 |

#### EXAMPLE 3

Each of the antifoggants (1), (2), (7) and (8) of this invention was incorporated in a sulfur- and gold-sensitized gelatin-silver iodobromide reversal color emulsion, respectively, and the resulting silver halide emulsions were applied to film bases and dried. The films were exposed on an NSC II-type sensitometer and processed in a hardening bath having the following composition for 3 minutes at 27° C.

|                      |          |
|----------------------|----------|
| Sodium Pyrophosphate | 20 g.    |
| Sodium sulfate       | 50 g.    |
| 37% Formaldehyde     | 17 ml.   |
| 10% sodium hydroxide | 1 ml.    |
| Water to make        | 1 liter. |

The light-sensitive films thus processed were washed with water for 4 minutes at 27° C. The films were then developed for 7 minutes at 27° C. in a developer having the following composition:

|                                 |          |
|---------------------------------|----------|
| N-methyl-p-aminophenol sulfate  | 1 g.     |
| Sodium Sulfite (anhydrous)      | 60 g.    |
| Hydroquinone                    | 10 g.    |
| Sodium carbonate (mono-hydrate) | 40 g.    |
| Potassium bromide               | 5 g.     |
| Potassium thiocyanate           | 1.5 g.   |
| 0.1% potassium iodide           | 5 ml.    |
| Water to make                   | 1 liter. |

The photographic properties of the thus developed photographic films were compared with those of a photographic film prepared and treated under the same conditions with the exception that an antifoggant of this invention was not added. The results obtained are shown in the following table and the results clearly show that fog-formation was prevented by the antifoggant of this invention.

| Concentration<br>(g./Ag 1 mol) | Relative<br>sensitivity | Fog  |
|--------------------------------|-------------------------|------|
| None (control)                 | 100                     | 0.85 |
| Antifoggant (1)                | 0.1                     | 0.67 |
| do                             | 0.2                     | 0.51 |
| Antifoggant (2)                | 0.4                     | 0.42 |
| do                             | 0.8                     | 0.28 |
| Antifoggant (7)                | 1.0                     | 0.35 |
| do                             | 2.0                     | 0.25 |
| Antifoggant (8)                | 2.0                     | 0.24 |
| do                             | 4.0                     | 0.13 |

## EXAMPLE 4

Each of the antifoggants (11), (12), (15) and (20) of this invention were incorporated in an aqueous 5 percent gelatin solution, respectively. A sulfur- and gold-sensitized gelatino silver iodo-bromide emulsion for use as a reversal color photographic material was coated on a glass plate of about 200 sq. cm., and dried. Then, 5 ml. of the gelatin solution prepared, as above was coated on the silver halide emulsion layer and dried. The thus double-coated photographic plates were exposed on an NSG II-type sensitometer and developed for 7 minutes at 27°C. in a developer having the same composition as in example 3.

The photographic properties of the photographic plates were compared with a plate which did not contain an antifoggant of this invention but which was otherwise identical. The results obtained were as follows:

|                  | Concentration (mg./5 ml. of 5% gelatin) | Relative sensitivity | Fog  |
|------------------|-----------------------------------------|----------------------|------|
| None (control)   |                                         | 100                  | 0.18 |
| Antifoggant (11) | 2.0                                     | 101                  | 0.16 |
| do               | 4.0                                     | 97                   | 0.14 |
| Antifoggant (12) | 20.0                                    | 98                   | 0.13 |
| do               | 40.0                                    | 94                   | 0.11 |
| Antifoggant (15) | 4.0                                     | 99                   | 0.15 |
| do               | 8.0                                     | 96                   | 0.13 |
| Antifoggant (20) | 4.0                                     | 100                  | 0.15 |
| do               | 8.0                                     | 95                   | 0.12 |

It is clear from the results in the table that the formation of fog was prevented by incorporation of an antifoggant of this invention in a protective layer for a silver halide emulsion layer without substantially reducing the sensitivity of the silver halide emulsion.

## EXAMPLE 5

Each of the antifoggants (14), (15), (18) and (19) of this invention were incorporated in a sulfur- and gold-sensitized gelatino-silver iodo-bromide emulsion for use as a reversal color photographic material. Each of the silver halide emulsions thus prepared was applied to a film base and dried. The photosensitive color films thus obtained were exposed and subjected to the following processings:

1. Prehardening 27°C. 3 minutes
2. Water rinsing 27°C. 4 minutes
3. Negative development 27°C. 7 minutes
4. Washing 27°C. 2 minutes
5. Reversal flash exposure 27°C.
6. Color development 27°C. 5 minutes
7. Water rinsing 27°C. 1 minute
8. Silver bleaching 27°C. 5 minutes
9. Fixing 27°C. 3 minutes
10. Water rinsing
11. Drying

The compositions of the processing baths used in the processings were as follows:

The composition of the hardening bath and the negative developer were the same as those in example 3.

## Color developing solution

|                                                    |          |
|----------------------------------------------------|----------|
| Sodium sulfide                                     | 5.0 g.   |
| N,N'-diethyl-p-phenylene-diamine hydrochloride     | 1.2 g.   |
| Sodium carbonate (monohydrate)                     | 20.0 g.  |
| Potassium bromide                                  | 0.3 g.   |
| 0.1% potassium iodide                              | 2.0 ml.  |
| 4-(p-toluene sulfonamido)-omega-benzoylacetanilide | 1.0 g.   |
| Sodium hydroxide                                   | 4.0 g.   |
| Water to make                                      | 1 liter. |

## Silver bleaching solution

|                        |          |
|------------------------|----------|
| Potassium ferricyanide | 60 g.    |
| Potassium bromide      | 20 g.    |
| Water to make          | 1 liter. |

Sodium thiosulfate 100 g.  
Sodium sulfite 15 g.  
Water to make 1 liter.

The photographic properties of the color photographic films obtained were compared with those of a film treated under the same conditions but containing no antifoggant of this invention. The results obtained are shown in the following table, in which the maximum density was measured by using a blue filter after color development.

|                  | Concentration (g./Ag 1 mol) | Maximum density |
|------------------|-----------------------------|-----------------|
| None (control)   | 2.0                         |                 |
| Antifoggant (14) | 0.4                         | 2.4             |
| do               | 0.8                         | 3.0             |
| Antifoggant (15) | 0.4                         | 2.3             |
| do               | 0.8                         | 2.6             |
| Antifoggant (19) | 1.0                         | 2.3             |
| do               | 2.0                         | 2.6             |

As shown in the above table, when the antifoggant of this invention was incorporated in the silver halide emulsion, the maximum density of the color image obtained was greatly increased due to the reduction in the formation of fog during negative development.

## EXAMPLE 6

25 The antifoggant (14) of this invention was added to samples of a sulfur and gold-sensitized gelatino-silver iodo-bromide emulsion for use as a negative color photographic material. 1-hydroxy-4-sulfo-2-n-octadecyl naphthamide was incorporated therein as a coupler by adding 20 parts by weight of an aqueous alkaline solution of the coupler (1 g. of the coupler per 1.4 mol of a 1N sodium hydroxide) to 100 parts by weight of the emulsion. The emulsion, after pH was adjusted to 7.0 with citric acid, was coated on a film base and dried.

30 The photosensitive color film thus obtained was exposed and developed using standard techniques in a color developer having the following composition:

N,N-diethyl-p-aminobenzoic acid 2.0 g.  
Sodium sulfite 2.0 g.  
Sodium carbonate (monohydrate) 50.0 g.  
Hydroxylamine hydrochloride 1.5 g.  
Potassium bromide 1.0 g.  
Water to make 1 liter.

The pH thereof was adjusted to  $10.8 \pm 0.1$  using NaOH.

45 The photographic film thus developed was further processed in a silver bleaching bath having the composition set out below and in a fixing bath having the composition set out below in order to remove the undeveloped silver halide and reduced silver:

| Bleaching solution         | 100 g.   |
|----------------------------|----------|
| Potassium ferricyanide     | 100 g.   |
| Potassium bromide          | 20 g.    |
| Water to make              | 1 liter. |
| Fixing solution            |          |
| Sodium thiosulfate         | 200 g.   |
| Sodium sulfite (anhydrous) | 20 g.    |
| 28% acetic acid            | 45 g.    |
| Boric acid                 | 7.5 g.   |
| Potassium alum             | 20 g.    |
| Water to make              | 1 liter. |

60 After this treatment, the density was measured using a red filter. The results obtained were compared with those obtained when a photographic material prepared under the same conditions with the exception that the antifoggant of this invention was not added. The results obtained are illustrated in the following table.

|                  | Concentration (g./Ag 1 mol) | Fresh |      | After aging <sup>3</sup> |      |
|------------------|-----------------------------|-------|------|--------------------------|------|
|                  |                             | A 1   | B 2  | A                        | B    |
| None (control)   |                             | 0.29  | 100  | 0.31                     | 100  |
| Antifoggant (14) |                             | 0.5   | 0.19 | 103                      | 0.16 |
|                  |                             | 1.0   | 0.13 | 100                      | 0.10 |
|                  |                             | 2.0   | 0.06 | 80                       | 0.06 |

<sup>1</sup> Cyan colored fog.

<sup>2</sup> Cyan relative sensitivity.

<sup>3</sup> After aging for 2 days at 50°C. and at 80% relative humidity.

From the above table, it is clear that the cyan colored fog was reduced while the sensitivity was not greatly decreased. The image obtained on the photographic material of this invention can be stored a long time, and it will remain stable.

## EXAMPLE 7

A dispersion of a coupler, 1-phenyl-3[3'(N-propyl-N-ocetylamo)-propioamide]-5-pyrazolone, was prepared by dissolving 5 g. of the coupler in 100 ml. of tricresyl phosphate. The solution was added to 100 g. of an aqueous 10 percent gelatin solution containing 8 ml. of an aqueous 5 percent solution of sodium dodecylbenzene sulfonate and stirred at 80-90° C. 10 Parts by weight of the dispersion thus prepared was added to 100 parts of a sulfur- and gold-sensitized gelatino-silver iodobromide emulsion. Antifoggant (2) of this invention was incorporated in the silver halide emulsion containing the coupler described above, and the resulting emulsion was coated on a film base and dried. The photosensitive color film thus obtained was exposed, color-developed by standard techniques in a color developer containing N,N-diethyl-p-aminobaniline, and then bleached and fixed to remove any undeveloped silver halide and reduced silver. The compositions of the color developer, bleaching solution and the fixing solution were same as those used in example 6.

After processing, the density was measured using a green filter.

The photographic film of this invention thus processed was compared with a control photographic film containing no antifoggant, and the results obtained were shown in the following table.

|                  | Concentration (g./Ag 1 mole) | Magenta-colored fog | Magenta relative sensitivity | Yellow         |                | Cyan |   | Magenta |   |
|------------------|------------------------------|---------------------|------------------------------|----------------|----------------|------|---|---------|---|
|                  |                              |                     |                              | A <sup>1</sup> | B <sup>2</sup> | A    | B | A       | B |
| None (control)   |                              | 0.13                | 100                          |                |                |      |   |         |   |
| Anti-foggant (2) | 1.0                          | 0.08                | 98                           |                |                |      |   |         |   |
|                  | 2.0                          | 0.06                | 87                           |                |                |      |   |         |   |

As shown in the above table, the formation of the magenta-colored fog was markedly prevented by the addition of the antifoggant, without substantial reduction in sensitivity.

## EXAMPLE 8

To 100 parts by weight of a sulfur- and gold-sensitized gelatino-silver chlorobromide emulsion there was added 40 parts by weight of a 5 percent aqueous alkaline solution of 3,5-dicarboxy-[4'-stearoylamido]benzoyl acetanilide. Antifoggant (1) of this invention was then incorporated in the emulsion. After adjusting the pH to 8.0, the resulting emulsion was coated on a film base to a thickness of 6 microns.

To 100 parts by weight of a sulfur-sensitized red-sensitive gelatino-silver chlorobromide emulsion there was added 10 parts by weight of a methanol solution of 0.25 percent 3'-allyl-6,7-benzo-3-ethyl-1,5'[2(1-ethyl-4-quinolinidene)ethylidene]-4'-oxa-thiazolinothiacyanine iodide and 25 parts by weight of a 5 percent aqueous alkaline solution of 1-hydroxy-2-n-octadecyl naphthamide. The pH was adjusted to 7.0, after incorporating antifoggant (1) of this invention into the silver halide emulsion. The thus prepared material was coated on the surface of the silver halide emulsion layer already formed at a thickness of 6 microns.

To 100 parts by weight of a sulfur-sensitized green-sensitive gelatino-silver chloride emulsion there was added 5 parts by weight of a 0.05 percent methanol solution of 3,3'-9-triethyl-5,5'-diphenyl-oxacarbocyanine rhodanide and 18 parts by weight of a 5 percent aqueous alkaline solution of 1-[3'-sulfo-4'-phenoxy]benzene]-3-heptadecyl-5-pyrazolone. The pH was then adjusted to 7.5. After incorporating antifoggant (1) of this invention into the silver halide emulsion thus prepared, the resultant material was further coated on the surface of the red-sensitive emulsion layer formed, as already described at a thickness of 6 microns.

The photosensitive color film thus prepared was exposed and subjected to the following processing:

|    |                     |        |            |
|----|---------------------|--------|------------|
| 5  | 1. Color developing | 20° C. | 10 minutes |
|    | 2. Water rinsing    | 20° C. | 2 minutes  |
|    | 3. Primary fixing   | 20° C. | 5 minutes  |
|    | 4. Water rinsing    | 20° C. | 5 minutes  |
|    | 5. Bleaching        | 20° C. | 5 minutes  |
|    | 6. Secondary fixing | 20° C. | 5 minutes  |
| 10 | 7. Water rinsing    | 20° C. | 10 minutes |

The compositions of the color developer, fixing solutions, and the bleaching solution used in the above processing were the same as those described in example 6.

After processing, the densities thereof were measured by using a blue filter, a green filter and red filter respectively.

The photographic color film of this invention thus processed was compared with a control film which contained no antifoggant in accordance with this invention. The results of this comparison are shown in the following table.

| Concentration of anti-foggant (1) (g./Ag one mol) | Yellow         |                | Cyan |      | Magenta |      |
|---------------------------------------------------|----------------|----------------|------|------|---------|------|
|                                                   | A <sup>1</sup> | B <sup>2</sup> | A    | B    | A       | B    |
| (b)                                               | (r)            | (g)            |      |      |         |      |
| 25                                                |                |                | 0.17 | 100  | 0.18    | 100  |
|                                                   | 1.0            |                | 0.14 | 103  | 0.17    | 98   |
|                                                   |                | 1.0            | 0.17 | 96   | 0.12    | 100  |
|                                                   |                |                | 1.0  | 0.16 | 101     | 0.16 |
|                                                   |                |                |      | 0.16 | 95      | 0.11 |
|                                                   |                |                |      | 0.13 | 93      | 0.10 |
|                                                   |                |                |      |      |         | 95   |

<sup>1</sup> Colored fog.

<sup>2</sup> Relative sensitivity.

NOTE: (b) a blue-sensitive emulsion layer; (r) a red-sensitive emulsion layer; (g) a green-sensitive emulsion layer.

As shown in the above table, the fog formation was remarkably reduced without substantially reducing the sensitivity.

When using other antifoggants which have the repeating units represented by general formula (1) other than the aforesaid antifoggants (1)-(20), almost identical results were obtained.

What is claimed is:

1. A photographic silver halide light sensitive element comprising a support having thereon a light sensitive silver halide emulsion layer which contains a compound having a repeating unit represented by the following formula



55 said compound containing at least four s-triazine rings in its molecule, and the amount of said compound being from about 0.01 g. to about 50 g. per 1 mole of silver halide in said emulsion layer, wherein R<sub>1</sub> represents a member selected from the group consisting of



60 65 -OR, and -SR, where R and R' each represent a member selected from the group consisting of (i) a hydrogen atom; (ii) an alkyl group having from 1-12 carbon atoms, a hydroxylalkyl group, a sulfoalkyl group, a salt thereof, a carboxyalkyl group, a salt thereof, and an aralkyl group, each of said groups having from 1-4 carbon atoms in the main straight carbon chain thereof; (iii) an unsubstituted aryl group having from 6-12 carbon atoms, an aryl group having from 6-12 carbon atoms substituted by a member selected from the group consisting of a sulfo group, a salt thereof, a sulfoxyl group, a salt thereof, a hydroxyl group, an alkyl group having from 1-4 carbon atoms,

an alkoxy group having from 1-4 carbon atoms, and a halogen atom; and unsubstituted cycloalkyl group, and a cycloalkyl group substituted by a member selected from the group consisting of a sulfo group, a salt thereof, a sulfoxyl group, a salt thereof, a hydroxyl group, each of said cycloalkyl groups having from 3-6 carbon atoms, an alkoxy group having from 1-4 carbon atoms, an alkoxy group having from 1-4 carbon atoms, and a halogen atom; and (iv) a pyridyl and a thiazolyl group; A represents a member selected from the group consisting of a polymethylene group having from 4-5 carbon atoms, and a polymethylene group having a heteroatomic group and forming a 5-6 membered ring together with a nitrogen atom; R<sub>2</sub>, R<sub>3</sub>, R<sub>4</sub> and R<sub>5</sub> each represent a member selected from the group consisting of a hydrogen atom, an alkyl group having from 1-4 carbon atoms and a hydroxyalkyl group; Y<sub>1</sub>, Y<sub>2</sub>, Y<sub>3</sub> and Y<sub>4</sub> each represent a member selected from the group consisting of a polymethylene group having from 2-12 carbon atoms, a polymethylene group having from 2-12 carbon atoms substituted by a member selected from the group consisting of an alkyl group having from 1-4 carbon atoms and a hydroxyalkyl group having from 1-4 carbon atoms, an arylene group having 6-12 carbon atoms, an arylene group having from 6-12 carbon atoms substituted by a member selected from the group consisting of a sulfo group, a salt thereof, a carboxyl group, a salt thereof, an alkyl group having from 1-4 carbon atoms, an alkoxy group having 1-4 carbon atoms and a halogen atom; Z represents a member selected from the group consisting of an oxygen atom, a sulfonyl group and a hydrocarbon residual group having from 1-2 carbon atoms; and k and m each represents 0 or 1.

2. A photographic silver halide light-sensitive element as claimed in claim 1 wherein R<sub>1</sub> is a member selected from the group consisting of

-OH, -OCH<sub>3</sub>, -OC<sub>2</sub>H<sub>5</sub>, -OC<sub>4</sub>H<sub>9</sub>



3. A photographic silver halide light-sensitive element as claimed in claim 1 wherein the atomic groups shown in said chemical formula as





5 4. A photographic silver halide light-sensitive element as claimed in claim 1, wherein said compound is a member selected from the group consisting of:

Wherein the number of S-triazine rings in the compound is:  $n$ .





5. A photographic silver halide light-sensitive element comprising a support having thereon a light-sensitive silver halide emulsion layer and a gelatin layer adjacent thereto, said gelatin layer containing a compound having a repeating unit represented by the following formula:



said compound containing at least 4s-triazine rings in its molecule, and the amount of said compound being from about 0.05 g. to about 250 g. per 1 Kg. of gelatin in said gelatin layer, wherein R, represents a member selected from the group consisting of



-OR, and -SR, where R and R' each represent a member selected from the group consisting of (i) a hydrogen atom; (ii) an alkyl group having from 1-12 carbon atoms, a hydroxyalkyl group, a sulfoalkyl group, a salt thereof, a carboxyalkyl group, a salt thereof, and an aralkyl group, each of said groups having from 1-4 carbon atoms in the main straight carbon chain thereof; (iii) an unsubstituted aryl group having from 6-12 carbon atoms, an aryl group having from 6-12 carbon atoms substituted by a member selected from the group consisting of a sulfo group, a salt thereof, a sulfoxyl group, a salt thereof, a hydroxyl group, an alkyl group having from 1-4 carbon atoms, an alkoxy group having from 1-4 carbon atoms, and a halogen atom; an unsubstituted cycloalkyl group, and a cycloalkyl group substituted by a member selected from the group consisting of a sulfo group, a salt thereof, a sulfoxyl group, a salt thereof, a hydroxyl group, each of said cycloalkyl groups having from 3-6 carbon atoms, an alkyl group having from 1-4 carbon atoms, an alkoxy group having from 1-4 carbon atoms, and a halogen atom; and (iv) a pyridyl and a thiazolyl group; A represents a member selected from the group consisting of a polymethylene group having from 4-5 carbon atoms, and a polymethylene group having a heteroatomic group and forming a 5-6 membered ring together with a nitrogen atom; R<sub>2</sub>, R<sub>3</sub>, R<sub>4</sub> and R<sub>5</sub> each represent a member selected from the group consisting of a hydrogen atom, an alkyl group having from 1-4 carbon atoms and a hydroxyalkyl group; Y<sub>1</sub>, Y<sub>2</sub>, Y<sub>3</sub> and Y<sub>4</sub> each represent a member selected from the group consisting of a polymethylene group having from 2-12 carbon atoms, a polymethylene group having from 2-12 carbon atoms substituted by a member selected from the group consisting of an alkyl group having from 1-4 carbon atoms and a hydroxyalkyl group having from 1-4 carbon atoms, an arylene group having 6-12 carbon atoms, an arylene group having from 6-12 carbon atoms substituted by a member selected from the group consisting of a sulfo group, a salt thereof, a carboxyl group, a salt thereof, an alkyl group having from 1-4 carbon atoms and a halogen atom, a cycloalkylene group having from 6-12 carbon atoms, and a cycloalkylene group having from 6-12 carbon atoms substituted by a member selected from the group consisting of a sulfo group, a salt thereof, a carboxyl group, a salt thereof, an alkyl group having from 1-4 carbon atoms, an alkoxy group having 1-4 carbon atoms and a halogen atom; Z represents a member selected from the group consisting of an oxygen atom, a sulfonyl group and a hydrocarbon residual group having from 1-2 carbon atoms; and k and m each represents 0 or 1.

6. A photographic silver halide light-sensitive element as claimed in claim 5 wherein  $R_1$  is a member selected from the group consisting of





8. A photographic silver halide light-sensitive element as claimed in claim 5, wherein said compound is a member selected from the group consisting of:

Wherein the number of S-triazine rings in the compound is: *n*.







30

35

40

45

50

55

60

65

70

75